

[54] LITH-TYPE SILVER HALIDE  
PHOTOGRAPHIC LIGHT-SENSITIVE  
MATERIAL

[75] Inventors: Yoshio Nishina; Teiji Habu; Tomio Nakajima; Akio Oshima; Eiichi Sakamoto; Noboru Fujimori; Kiyomitsu Mine; Hiroo Toya, all of Hino, Japan

[73] Assignee: Konishiroku Photo Industry Co., Ltd., Tokyo, Japan

[21] Appl. No.: 822,601

[22] Filed: Aug. 8, 1977

## Related U.S. Application Data

[63] Continuation of Ser. No. 613,628, Sep. 15, 1975, abandoned.

## [30] Foreign Application Priority Data

Sep. 24, 1974 [JP] Japan 49/07314

[51] Int. Cl.<sup>2</sup> G03C 5/04; G03C 1/18; G03C 1/06

[52] U.S. Cl. 96/27 E; 96/33; 96/95; 96/137

[58] Field of Search 96/27 H, 27 E, 137, 96/95, 33

## [56] References Cited

## U.S. PATENT DOCUMENTS

|           |         |                 |         |
|-----------|---------|-----------------|---------|
| 3,232,761 | 2/1966  | Allen           | 96/66 R |
| 3,775,111 | 11/1973 | Norman          | 96/27 H |
| 3,775,114 | 11/1973 | Gracia et al.   | 96/33   |
| 3,867,146 | 2/1975  | Nakazawa et al. | 96/27 H |
| 3,895,948 | 7/1975  | Shiba et al.    | 96/95   |

3,915,713 10/1975 Shiba et al. 96/95

## OTHER PUBLICATIONS

J. Opt. Soc. Am., vol. 53, No. 12, Dec. 1963, pp. 1377-1381.

Applied Optics, Nov. 1969, vol. 8, No. 11, pp. 2353-2354.

Data Release, Eastman Kodak, 1969, pp. 1-10.

Primary Examiner—Mary F. Kelley  
Attorney, Agent, or Firm—Bierman & Bierman

[57]

## ABSTRACT

A lith-type silver halide photographic light-sensitive material for forming halftone dot images is disclosed which contains a sensitizing dye represented by the following general formula:



wherein  $Z_1$  is an atomic group necessary for forming a naphthothiazole ring,  $Z_2$  is an atomic group necessary for forming a member selected from a group consisting of substituted or unsubstituted, benzothiazole, benzoselenazole, naphthothiazole and naphthoselenazole nucleus,  $R_1$  and  $R_2$  are respectively a substituted or unsubstituted alkyl group,  $X^\ominus$  is an anion, and  $n$  is a positive integer of 1 or 2 with the proviso that when the dye is an inner salt,  $n$  is 1.

1 Claim, No Drawings

## LITH-TYPE SILVER HALIDE PHOTOGRAPHIC LIGHT-SENSITIVE MATERIAL

This is a continuation application of Ser. No. 613,628 filed Sept. 15, 1975 now abandoned and which claims the priority of Japanese Patent Application No. 107314/1974 filed on Sept. 17, 1974.

### DETAILED DESCRIPTION OF THE INVENTION

This invention relates to a lith-type silver halide photographic light-sensitive material for forming halftone dot images by the scanner process using neon-helium laser beams as light source. More particularly, the invention relates to such lith-type silver halide photographic light-sensitive material which comprises a silver halide emulsion containing 60 to 90 chloride, 10 to 40 bromide and less than 5 mole percent iodide, has a high sensitivity to a wave length inherent of neon-helium laser beams, namely a wave length of 6328 nm, and exhibits excellent in reciprocity law failure and dot image-forming property at high-illuminance and short-time exposure less than  $10^{-4}$  second.

A so-called scanner process for forming images by scanning an original, light-exposing a silver halide photographic photosensitive material based on the resulting image signal and thus forming a negative or positive image corresponding to the original image is known in the art. This scanner process is divided into two types. According to one type, an ordinary silver halide photographic light-sensitive material is used to form an image having a continuous gradation and according to the other type a lith-type silver halide photographic light-sensitive material is used to obtain a halftone dot image. In industries of printing and photo-engraving, the latter process is now used more frequently than the former process because the latter process provides sharp images excellent in the resolving power and the engraving process can be shortened to enable labor-saving. The scanner process forming halftone dot images is divided in a so-called dot generating system for forming halftone dots by using a dot generator and a system for forming halftone dots by using a contact screen. As the light source for a dot-generating machine used in these systems (for example, electronic direct color-scanner), there have heretofore been mainly used a glow-discharge lamp, a xenon lamp, a mercury lamp and the like. However, each of these light sources involves practical difficulties, because of a relatively low power and a relatively short life. Recently, use of coherent laser beams as light source has been tried and halftone dot-generating machines including this light source have been developed.

As the medium for generator of laser beam, there are employed ruby, neon-helium gas, argon gas, krypton gas, cadmium gas, carbon dioxide gas and the like. A laser beam generator using neon-helium gas are employed most broadly, because they are cheaper than other generator and stable outputs can be obtained.

A wave length of laser beams generated by a neon-helium laser is 6328 nm. Accordingly, lith-type silver halide photographic light-sensitive materials to be used for forming halftone dot images by employing an electronic direct color-scanner are required to have a high sensitivity to a wave length of 6328 nm and an excellent adaptability to high-illuminance short-time exposure (especially one conducted for less than  $10^{-4}$  second) which is an indispensable requirement for formation of

halftone dots according to the scanner process. However, conventional lith-type silver halide photographic light-sensitive materials do not always possess a sufficient sensitivity to neon-helium laser beams, exhibit remarkable reciprocity failure at the high-illuminance short-time exposure and are insufficient in the dot quality. Accordingly, none of now available lith-type silver halide photographic light-sensitive materials can be practically used for formation of halftone dot images according to the scanner process.

It is therefore a primary object of this invention to provide a lith-type silver halide photographic light-sensitive material for forming halftone dot images according to the scanner process using neon-helium laser beams as light source, which has a high sensitivity to a wave length of 6328 nm inherent of neon-helium laser beams and is excellent in reciprocity law failure at the high-illuminance short-time exposure (especially one conducted for less than  $10^{-4}$  second) and in dot quality.

It has been found that the foregoing object can be attained by sensitizing a silver halide by incorporating a carbocyanine sensitizing dye represented by the following general formula into a lith-type silver halide photographic light-sensitive material:



In the above general formula,  $\text{Z}_1$  stands for a group of atoms necessary for formation of a naphthothiazole ring, and  $\text{Z}_2$  stands for a group of non-metallic atoms necessary for formation of an substituted or unsubstituted benzthiazole, benzselenazole, naphthothiazole or naphthoselenazole nucleus. As the benzthiazole nucleus, there can be mentioned, for example, nuclei of benzthiazole, 5-chlorobenzthiazole, 5-methylbenzthiazole, 5-methoxybenzthiazole, 5-hydroxybenzthiazole, 5-hydroxy-6-methylbenzthiazole, 5,6-dimethylbenzthiazole, 5-phenylbenzthiazole, 5-carboxybenzthiazole, 5-ethoxycarbonylbenzthiazole, 5-dimethylaminobenzthiazole and 5-acetylaminobenzthiazole. As the benzselenazole nucleus, there can be mentioned, for example, nuclei of benzselenazole, 5-chlorobenzselenazole, 5-methylbenzselenazole, 5-methoxybenzselenazole, 5-hydroxybenzselenazole, 5,6-dimethylbenzselenazole, 5,6-dimethoxybenzselenazole, 5-ethoxy-6-methylbenzselenazole, 5-hydroxy-6-methylbenzselenazole and 5-phenylbenzselenazole. As the naphthothiazole nucleus, there can be mentioned, for example, nuclei of  $\beta$ -naphthothiazole and  $\beta,\beta$ -naphthothiazole. As the naphthoselenazole nucleus, there can be mentioned, for example, a nucleus of  $\beta$ -naphthoselenazole.  $\text{R}_1$  and  $\text{R}_2$  stand for a lower alkyl group or a substituted lower alkyl group. As specific examples of  $\text{R}_1$  and  $\text{R}_2$ , there can be mentioned methyl, ethyl, n-propyl,  $\beta$ -carboxyethyl,  $\gamma$ -sulfopropyl,  $\gamma$ -sulfonylpropyl,  $\delta$ -sulfonylpropyl and sulfoethoxyethyl groups.  $\text{X}^\ominus$  designates an anion such as a halogen ion, a perchloric ion, thiocyanic ion, a benzene-sulfonic ion, a p-toluenesulfonic ion and a methylsulfuric ion, and  $n$  is a positive integer of 1 or 2 with the proviso that when the dye is an inner salt,  $n$  is 1.

The sensitizing dye of this invention is a thiacyanine or selenacarbocyanine having an ethyl group substituted at the meso-position of the trimethine chain, and the sensitizing dye has a J-band sensitizing property which is advantageous for spectral sensitization in a specific wave length region.

Typical instances of the sensitizing dye of this invention will now be illustrated.



-continued  
[Illustrative Sensitizing Dyes]

(14)



(15)



(1)

(2)

(3)

(4)

(5)

(6)

(7)

(8)

(9)

(10)

(11)

(12)

(13)

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

isocyanate and cysteine, active or inactive selenium sensitizers, gold compounds, e.g., potassium chloroaurate, auric trichloride, potassium auric thiocyanate and 2-aurothiabenzthiazole methylchloride, palladium compounds, e.g., ammonium chloropalladate and sodium chloropalladite, platinum compounds, e.g., potassium chloroplatinate, ruthenium compounds, rhodium compounds, and other novel metal sensitizing agents, e.g., iridium compound. These sensitizing agents can be used singly or in the form of a mixture of two or more of them. Further, the emulsions may be sensitized by reducing agents as well as the foregoing chemical sensitizing agents. Moreover, the emulsions may be stabilized by a triazole, an imidazole, an azaindene compound, a benzthiazolium compound, a zinc compound, a cadmium compound, a mercaptan or a mixture thereof. Still further, the emulsions may be sensitized by a thioether type quaternary ammonium salt or the like. Still in addition, if desired, the high-illuminance characteristic of the emulsions can be improved by using a pyrazolone compound disclosed U.S. Pat. No. 3,594,173, or the dot-forming characteristic of the emulsions may be improved by addition of a polyalkylene oxide compound.

Moreover, swelling agents, plasticizers and film property-improving agents such as glycerin, dihydroxyalkanes, e.g., 1,5-pentane diol, esters of ethylene-bis-glycolic acid, bis-ethoxydiethylene glycol succinate and water-dispersible particulate polymeric compounds formed by emulsion polymerization may be incorporated in the emulsions. Furthermore, film-hardening agents such as ethylene-imine type compounds, dioxane derivatives, hydroxypolysaccharides, dicarboxylic chlorides and diesters of methanesulfonic acid, coating assistants such as saponin and sulfosuccinic acid salts, fluorescent whitening agents, surfactants, anti-staining agents and other photographic additives. Still in addition, the emulsions may be sensitized by a sensitizing dye other than the dye represented by the above general formula, such as a cyanine dye, merocyanine dye and a composite cyanine dye.

Still further, in order to improve the stability to dark room rays, for example, a compound disclosed in Japanese Patent Application Laid-Open Specification No. 60918/73, may be incorporated as a photographic dye into the emulsions.

This invention will now be illustrated in detail by reference to the following Examples that by no means limit the scope and embodiments of this invention.

#### EXAMPLE 1

A methanol solution of a sensitizing dye of this invention was incorporated into a silver chlorobromide (comprising 80 mole % of silver chloride and 20 mole % of silver bromide) emulsion prepared by a known method, prior to coating in such an amount that the content of the sensitizing dye was 150 mg per mole of the silver halide, and known additives necessary for photographic materials were further added to the emulsion, to thereby from a lith-type silver halide photographic emulsion. For comparison, emulsions were similarly prepared by using the following comparative sensitizing dyes.

Each of the so prepared emulsions was coated and dried on a polyethylene terephthalate film to obtain a sample.



The so prepared samples were exposed to light according to the following two methods:

#### Method (1)

A gray contact screen (50 lines/inch; manufactured by Dainippon Screen) was placed in the state contacting closely to the sample, and light exposure was carried out for 2 seconds through an ordinary light wedge by using a sensitometer (tungsten rays of 2854° D) and an interference filter allowing passage of red light of a wave length of 631.5nm.

#### Method (2)

A gray contact screen (150 lines/inch; manufactured by Dainippon Screen) was placed in the state contacting closely to the sample, and light exposure was conducted for 1/10000 second by using a neon-helium laser generator (Gas Laser GLS 2004 manufactured by Nippon Denki Kabushiki Kaisha) and a neutral gray wedge.

Exposure amount was adjusted by the neutral gray filter so that it was maintained at the same level in both the methods (1) and (2).

After the above exposure, development was carried out by using a lith-type developer having the following composition and the sensitivity and dot quality at the optimum time point (the time of development required for obtaining sharpest dots) were determined.

In the case of the light exposure method (2) the optimum development time appeared very slightly later than in the case of the method (1), but since this time lag was within several seconds, no disadvantage was brought about even when evaluation was made based on the same development time. Composition of Developer (development was conducted at 27° C.):

|                                     |         |
|-------------------------------------|---------|
| hydroquinone                        | 16 g    |
| formaldehyde sodium hydrogensulfite | 50 g    |
| sodium sulfite                      | 2 g     |
| potassium bromide                   | 1 g     |
| sodium carbonate (monohydrate)      | 60 g    |
| triethylene glycol                  | 40 g    |
| water                               | balance |
| total                               | 1000 ml |

Results of measurement of the photosensitivity and dot quality of the developed samples are as shown in Table 1.

In the Table, values of the relative sensitivity are relative values based on the sensitivity (100) of the comparative sensitizing dye [A] observed in the interference filter light-exposure method [method (1)]. The dot quality was evaluated based on the sharpness of the dot silver image observed under a microscope according to the 5-graduated scale in which point "1" was given to the worst image and point "5" was given to the best image.

Table 1

| Used Compound | Exposed by Method (1) |             | Exposed by Method (2) |             | Optimum Point (Development Time) |
|---------------|-----------------------|-------------|-----------------------|-------------|----------------------------------|
|               | Relative Speed        | Dot Quality | Relative Speed        | Dot Quality |                                  |
| 1             | 110                   | 3           | 115                   | 4           | 97                               |
| 2             | 125                   | 4           | 125                   | 5           | 95                               |
| 5             | 120                   | 4           | 120                   | 5           | 98                               |
| 7             | 105                   | 4           | 110                   | 5           | 100                              |
| 8             | 115                   | 3           | 115                   | 4           | 95                               |
| 13            | 125                   | 4           | 125                   | 5           | 95                               |
| A             | 100                   | 3           | 92                    | 2           | 130                              |
| B             | 90                    | 4           | 90                    | 2           | 100                              |
| C             | 100                   | 3           | 80                    | 2           | 150                              |
| D             | 85                    | 3           | 80                    | 1           | 130                              |

As is seen from the results shown in Table 1, lith-type films containing a sensitizing dye of this invention exhibit higher sensitivity and better dot quality when exposed according to the neon-helium laser beam exposure method [method (2)] than when exposed according to the interference filter exposure [method (1)].

It is also seen that sensitizing dyes of this invention are much excellent over the comparative sensitizing dyes in photographic characteristics. What must be noted is that even if no substantial difference of the sensitivity is brought about by the difference of the light exposure method, a distinct difference of the dot quality is observed between the sensitizing dyes of this invention and the comparative sensitizing dyes when the high-illuminance short-time exposure is carried out by using coherent laser beams.

#### EXAMPLE 2

Samples prepared in the same manner as described in Example 1 were exposed to neon-helium laser beams having an output of 2 nW and developed by using the same liquid developer as used in Example 1 while changing the developing time.

Dot silver images were examined under a microscope, and the optimum development time (optimum point) required for obtaining sharpest images was determined with respect to each sample to obtain results shown in Table 2.

Table 2

| Used Compound | Optimum Point (Development Time) | Dot Quality |
|---------------|----------------------------------|-------------|
| 1             | 95                               | 4           |
| 2             | 95                               | 5           |
| 3             | 97                               | 4           |
| 4             | 94                               | 4           |
| 5             | 100                              | 5           |
| 10            | 95                               | 5           |
| 15            | 97                               | 4           |
| A             | 130                              | 3           |
| B             | 100                              | 3           |
| C             | 150                              | 2           |
| D             | 130                              | 3           |

As is apparent from the results shown in Table 2, lith-type films containing a sensitizing dye of this invention exhibit better dot quality than that obtained from

lith-films containing the comparative sensitizing dye [A], [B], [C] or [D].

What is claimed is:

1. A method of forming halftone dot images comprising imagewise exposing a photographic light sensitive material with neon helium laser beams, and developing said exposed photographic light sensitive material with an infectious developer, said photographic light sensitive material comprising a silver halide emulsion wherein said silver halide contains 60 to 90 mole percent of silver chloride, 10 to 40 mole percent of silver bromide and less than 5 mole percent of silver iodide, and a sensitizing dye selected from the group consisting of:



-continued



(13)



(12)

(14)

10



\* \* \* \* \*

15

20

25

30

35

40

45

50

55

60

65

UNITED STATES PATENT OFFICE  
CERTIFICATE OF CORRECTION

PATENT NO. : 4,121,935  
DATED : October 24, 1978  
INVENTOR(S) : Yoshio Nishina, et al

It is certified that error appears in the above-identified patent and that said Letters Patent are hereby corrected as shown below:

On Page 1, an error was made at line [30] and should read as follows:

[30] Foreign Application Priority Data  
Sep. 17, 1974 [JP] Japan..... 49-107314

Signed and Sealed this  
*Twentieth Day of February 1979*

[SEAL]

*Attest:*

RUTH C. MASON  
*Attesting Officer*

DONALD W. BANNER  
*Commissioner of Patents and Trademarks*